

Dec. 30, 1969

J. RAGUIN ET AL

3,486,882

CONTINUOUS STEEL MAKING PROCESS

Filed July 23, 1968

2 Sheets-Sheet 1



Dec. 30, 1969

J. RAGUIN ET AL

3,486,882

CONTINUOUS STEEL MAKING PROCESS

Filed July 23, 1968

2 Sheets-Sheet 2



FIG. 2

1

3,486,882

**CONTINUOUS STEEL MAKING PROCESS**  
Jean Raguin and Jean Rouquet, Metz, Moselle, France, assignors to Institut de Recherches de la Siderurgie Francaise, Saint Germain-en-Laye, Yvelines, France  
Continuation-in-part of application Ser. No. 515,807, Dec. 12, 1965. This application July 23, 1968, Ser. No. 753,336  
Claims priority, application France, Dec. 24, 1964, 999,972  
Int. Cl. C21c 5/00, 7/00  
U.S. Cl. 75—51

15 Claims

## ABSTRACT OF THE DISCLOSURE

A method for continuously producing steel in which a solid prereduced steel-forming material is continuously introduced into a refining vessel containing molten steel and slag while simultaneously and continuously introducing thermogenic material and gaseous oxygen in such amounts into the refining vessel and the molten mass therein that the amount of thermogenic material by exothermic reaction with the oxygen will insure melting of the introduced prereduced solid steel-forming material and the amount of gaseous oxygen is sufficient to convert said prereduced steel-forming material into steel to thus obtain in the vessel a mixture of molten steel and slag. The gaseous oxygen is introduced into the vessel from above in form of a jet so as to transform part of the mixture into a metal-slag foam which is continuously withdrawn by overflow from the refining vessel at such a rate that the amount of molten mass therein remains substantially constant.

## CROSS-REFERENCES TO RELATED APPLICATIONS

The present application is a continuation-in-part application of the application Ser. No. 515,807, filed Dec. 12, 1965 and now abandoned.

## BACKGROUND OF THE INVENTION

The present invention relates to a process of making steel and, more particularly, the present invention is concerned with a process of making steel which requires only one melting of the steel-forming raw material.

The present invention is specifically concerned with making steel from prereduced, solid, steel-forming material.

It is an object of the present invention to produce liquid steel in a continuous manner from prereduced solid, steel-forming material.

It is a further object of the present invention to produce steel from such prereduced, solid, steel-forming materials in a simple economical manner.

Other objects and advantages of the present invention will become apparent from a further reading of the description and of the appended claims, and it will be noted that according to the present invention iron ore may be converted into steel without requiring the intermediate production of pig iron.

## SUMMARY OF THE INVENTION

With the above and other objects in view, the present invention relates to a method of continuously producing steel comprising the steps of continuously introducing into a refining vessel, containing a mixture of molten steel-forming materials, a solid prereduced steel-forming

2

material at an elevated temperature below the melting point of the prereduced material, simultaneously and continuously introducing thermogenic material and gaseous oxygen respectively in such amounts into the refining vessel and the molten mass therein so that the amount of thermogenic material by exothermic reaction with the oxygen will insure melting of the simultaneously and continuously introduced steel forming material and that the amount of the simultaneously introduced oxygen is sufficient to convert the continuously introduced prereduced steel-forming material into steel to thus obtain in the vessel a mixture of molten steel and slag. The gaseous oxygen is introduced in a jet from above into the mixture in the refining vessel to transform at least part of the mixture in the refining vessel into a metal-slag foam, and continuously withdrawing by overflow the metal-slag foam from the refining vessel at such a rate that the amount of molten mass in the refining vessel remains substantially constant.

20 Within the context of the present specification and claims, the term "prereduced solid material" is intended to denote iron ores which have been submitted to a reducing treatment such that between about 40 and 100% of the bound oxygen of the iron ore will have been removed 25 by means of reducing agents such as, for instance, carbon. If for the purpose of producing the prereduced solid material an excess amount of carbon or the like is applied, such excess amount may be retained in the prereduced solid material which is introduced into the refining vessel. 30 The other components of the iron ore and such also of the prereduced solid material may vary greatly.

Process of manufacturing such prereduced solid materials are well known in the art and are described for instance in a publication of CECA (Communaute Européenne Charbon Acier), entitled "Etude bibliographique des Procedes de reduction directe des minerais de fer," dated December 1960. Therein, the DLM, Freeman, Wi-berg and Finsider processes are described.

40 The term "thermogenic materials" is to be understood, in the context of the present specification and claims, as denoting materials which react in an exothermic manner with oxygen or oxidizing substances. The amount of thermogenic material which is to be simultaneously introduced with the prereduced solid material, in accordance 45 with the present invention, must be such that the heat requirements of the process are supplied by the heat provided by the enthalpy of the prereduced material, which depends on the temperature at which the prereduced material is introduced into the refining vessel (which temperature preferably will be an elevated temperature below the melting point of the prereduced material), the enthalpy of the thermogenic material and the heat formed by oxidation of the same, and the combustion heat of gases which are oxidized during the refining process, primarily the combustion of CO into CO<sub>2</sub>.

50 Elements which form part of the thermogenic material and which may be oxidized in an exothermic reaction include, for instance, carbon, silicon and phosphorus.

55 The heat which is thus made available must be sufficient to balance the thermic losses which correspond to the enthalpy of the slag, the enthalpy of the withdrawn molten steel, the enthalpy of the gases, and other thermic losses due to radiation, etc.

60 According to various preferred embodiments of the present invention, the above described process may comprise one or more of the following features:

(a) Prereduced steel-forming material may be introduced in the form of pellets, generally having a size of

between 2 and 40 mm. and preferably between 10 and 20 mm.

(b) The solid prerduced steel-forming material may be introduced in pulverulent form, for instance having a particle size of between 10 microns and 2 mm. and preferably having a particle size between 100 microns and 1 mm.

(c) The prerduced solid steel-forming material may be sponge iron and, preferably, the particle size of the sponge iron may be greatly reduced and a pulverulent mass of sponge iron introduced into the refining vessel.

(d) A strongly thermogenic material such as, for instance, coke may be additionally, simultaneously with the prerduced material, and continuously introduced into the refining vessel.

(e) The solid prerduced steel-forming material and the thermogenic material may be jointly introduced into the refining vessel in the form of a mixture of these two types of materials.

(f) The thermogenic material may be introduced pneumatically in pulverulent form, for instance in the form of a pulverulent suspension of thermogenic material in a suitable carrier gas.

(g) At least a portion of the gas produced during the refining process within the molten metal mass in the refining vessel may be oxidized and burned by reaction with a portion of the oxygen introduced into the molten metal, before the gas reaches the upper level of the mass of molten metal in the refining vessel.

It will be understood, that the process of the present invention is primarily concerned with a method of directly refining prerduced solid steel-forming materials which are introduced in hot condition into a refining vessel wherein the prerduced solid materials are changed into a liquid melt. These prerduced steel-forming materials may contain, in addition to iron, thermogenic elements such as carbon, phosphorus or silicon in amounts sufficient to provide, upon reaction of these thermogenic materials with oxygen, in part or fully the heat necessary for the melting of the material and for transformation of the same into steel. If the amount of thermogenic materials contained in the prerduced solid material does not suffice for creating the amount of heat required for the process then, as described further above, thermogenic materials are additionally introduced into the refining vessel.

It is preferred according to the present invention to introduce the predeuced, solid steel-forming material into the refining vessel, and into the molten steel bath contained therein, in the form of pellets which, due to their geometrical shape, are particularly suitable for being introduced in a regular and controllable flow so that within given time periods the same amounts of prerduced, solid steel HY forming material are introduced into the refining vessel.

According to another preferred embodiment, the prerduced, solid, steel-forming material is introduced in pulverulent form, by being blown into the refining vessel suspended in a hot reducing gas. This is particularly advantageous if the prerduced material is obtained in pulverulent form, for instance by fluidization processes known, per se, to those skilled in the art. The hot reducing gas serving as carrier for the pulverulent, prerduced, steel-forming material may also be derived from the waste gas leaving the refining vessel.

The present invention also contemplates, as discussed further above, the simultaneous introduction of solid, strongly thermogenic materials, which, for instance may be carbon in the form of coke or graphite, phosphorus in the form of ferrophosphorus, silicon in the form of ferrosilicon and aluminum in the form of ferroaluminum.

It is also within the scope of the present invention to reach a portion of the refining gas which develops in the metal bath immediately, and prior to escape of such refining gas from the metal bath, with oxygen so as to con-

vert the refining gas to carbon dioxide, since thereby the heat content of the molten metal bath may be significantly increased.

The novel features which are considered as characteristic for the invention are set forth in particular in the appended claims. The invention itself, however, both as to its construction and its method of operation, together with additional objects and advantages thereof, will be best understood from the following description of specific embodiments when read in connection with the accompanying drawings in which the drawing is a schematic elevational view of an apparatus for carrying out the present invention.

The invention will now be described by way of the following example with reference to the drawing without, however, limiting the invention to the specific details of the example.

#### BRIEF DESCRIPTION OF THE DRAWING

FIG. 1 is a schematic view showing an arrangement for carrying out the method of the present invention; and FIG. 2 is a view of an embodiment thereof.

#### DESCRIPTION OF THE PREFERRED EMBODIMENTS

Referring now to the drawing, reference numeral 1 indicates a heat insulated hopper made of refractory bricks and containing a relatively small amount of prerduced, hot, solid, steel-forming pellets which are introduced into hopper 1 in a continuous manner from a conventional pelletizing device (not shown). The pellets may be produced in any conventional manner and producing of the pellets does not form part of the present invention.

From hopper 1, the mass of pellets is then continuously and evenly introduced through a refractory conduit 3 into a continuous refining vessel 2 containing molten steel in its lower portion. The rate of introduction of pellets into a refining vessel 2 is controlled by means of a conventional, revolving distributor wheel 4.

A stream of oxygen under pressure having pulverulent lime suspended therein is introduced into refining vessel 2 from above in form of a jet through lance 5 projecting into the reforming vessel and being adjustable in vertical direction. It will be seen that although the nozzle of downwardly directed lance 5 is located above the upper level of the molten metal, nevertheless, oxygen gas will be blown into the interior of the molten metal mass. The thus introduced oxygen gas will assure the refining of the prerduced material and the excess heat of the refining reaction will bring about the melting of the pellets to thus form a mixture of refined metal and at least part of which is transformed by the oxygen jet into a slag-metal foam which passes by overflowing into portion 6

of the refining vessel in which the two phases, namely the slag and the molten steel, are allowed to separate into a continuous metal phase and a slag phase floating thereon. The molten steel is then removed through an opening 7 located in the bottom of vessel portion 6, while the supernatant slag flows through an opening 8 in the side wall of vessel portion 6.

The pellets of pulverulent prerduced products which are introduced into the left hand or refining portion of refining vessel 2 are preheated, prior to introduction into the vessel 2, preferably to a temperature of about 700° C. and have the following composition:

|                                                  | Percent |
|--------------------------------------------------|---------|
| Fe, metallic                                     | 73.8    |
| Fe, total                                        | 80.8    |
| CaO                                              | 0.45    |
| SiO <sub>2</sub>                                 | 3.6     |
| MgO                                              | 1.8     |
| Al <sub>2</sub> O <sub>3</sub>                   | 0.9     |
| C                                                | 10.0    |
| 75 Miscel. (P <sub>2</sub> O <sub>5</sub> , MnO) | 0.35    |

118 standard cubic meters of oxygen carrying suspended therein 117 kg. of pulverulent lime, are blown into the refining portion of refining vessel 2 through lance 5 per 1000 kg. of prereduced, solid steel-forming material.

In this manner, raw steel is obtained having a temperature of 1600° C. and the following composition:

|    | Percent |
|----|---------|
| C  | 0.040   |
| P  | 0.005   |
| S  | 0.006   |
| Mn | 0.050   |

Thereby, an amount of 270 kg. of slag is formed per 1000 kg. of prereduced steel-forming pellets, which slag has the following composition:

|                                | Percent |
|--------------------------------|---------|
| CaO                            | 45      |
| FeO                            | 30      |
| SiO <sub>2</sub>               | 12      |
| Al <sub>2</sub> O <sub>3</sub> | 4       |
| MgO                            | 7       |
| Miscel.                        | 2       |

According to FIG. 2 a lance 11 is provided in the vicinity of lance 5 for the purpose of introducing into refining vessel 2 a suspension of a mixture of prereduced steel-forming material in form of pulverulent sponge iron and of thermogenic material the latter consisting, for instance, of a mixture of pulverulent coke and pulverulent ferrosilicon containing 90% silicon.

It is obvious that the lance 11 could be used in the arrangement of FIG. 1 to introduce separately the thermogenic material in pulverulent form, and that any combination of introducing means of the prereduced material and thermogenic material is possible. For instance pulverulent coke could be introduced through lance 11 and ferrosilicon in grains and prereduced ore through hopper 1.

The gases which are formed in refining vessel 2, and particularly in the portion thereof into which lances 5 and 11 extend, are withdrawn through flue 9. An additional lance 10 serves for introducing oxygen into the interior of vessel 2, again above the reacting mass of prereduced material, for the purpose of causing at least partial combustion of combustible refining gases emanating from the molten turbulent metal mass in the left hand portion of the refining vessel.

Pulverulent sponge iron which is introduced into the left hand of refining vessel 2 is preheated, prior to the introduction in the vessel, preferably to a temperature of about 750° C. and has the following composition.

|           | Percent |
|-----------|---------|
| Fe, metal | 88      |
| Fe, total | 94.5    |
| Gangue    | 5.5     |

The gases which escape from the refining vessel and which are subjected to partial combustion by means of the oxygen from lance 10 have a temperature of 1600° C. and consist of 21.9% CO<sub>2</sub> and 78.1% CO.

Without further analysis, the foregoing will so fully reveal the gist of the present invention that others can by applying current knowledge readily adapt it for various applications without omitting features that, from the standpoint of prior art, fairly constitute essential characteristics of the generic or specific aspects of this invention and, therefore, such adaptations should and are intended to be comprehended within the meaning and range of equivalence of the following claims.

What is claimed as new and desired to be secured by Letters Patent is set forth in the appended claims:

1. A method of continuously producing steel comprising the steps of continuously introducing into a refining vessel containing a mass of molten steel and slag a solid prereduced steel-forming material at an elevated temperature below the melting point of said material; simultane-

70  
75

ously and continuously introducing thermogenic material and gaseous oxygen respectively in such amounts into the refining vessel and the molten mass therein so that the amount of thermogenic material by exothermic reaction with the oxygen will insure melting of the simultaneously and continuously introduced steel-forming material and that the amount of the simultaneously introduced oxygen is sufficient to convert the continuously introduced prereduced steel-forming material into steel to thus obtain in the vessel a mixture of molten steel and slag, said gaseous oxygen being introduced in a jet from above into the material in the refining vessel to transform at least part of the mixture in said refining vessel into a metal-slag foam; and continuously withdrawing by overflow said metal-slag foam from said metal refining vessel at such a rate that the amount of molten mass in said refining vessel remains substantially constant.

2. A method as defined in claim 1, wherein said metal slag foam is withdrawn into a decanting vessel and including the steps of causing in said decanting vessel separation of said metal-slag foam into a continuous metal phase and a slag phase floating thereon, and separately discharging in the slag phase and the continuous metal phase from said decanting vessel.

3. A method as defined in claim 2, wherein said thermogenic material is selected from the group consisting of carbon, ferrophosphorus, ferrosilicon and ferroaluminum.

4. A method as defined in claim 3, wherein said thermogenic material is coke.

5. A method as defined in claim 3, wherein said thermogenic material is continuously introduced into the refining vessel admixed to said prereduced material.

6. A method as defined in claim 3, wherein said thermogenic material is continuously introduced into said refining vessel in the form of a pulverulent suspension thereof in a carrier gas.

7. A method as defined in claim 6, wherein said carrier gas with said thermogenic material in pulverulent form suspended therein is blown in a jet from above into said mass of molten material in said refining vessel.

8. A method as defined in claim 2, wherein said solid prereduced material is continuously introduced into said refining vessel in the form of pellets.

9. A method as defined in claim 8 wherein said pellets contain thermogenic material in sufficient amount to provide the heat necessary for the melting of said pellets and for their transformation into steel.

10. A method as defined in claim 2, wherein said solid prereduced material is in pulverulent form.

11. A method as defined in claim 2, wherein said solid prereduced material is sponge iron.

12. A method as defined in claim 2, wherein oxidizable gas is formed during transformation of said solid prereduced material into steel, and wherein at least a portion of said oxidizable gas is reacted with oxygen while still below the upper level of said mass of molten steel in said refining vessel.

13. A method as defined in claim 2, wherein combustible gas is formed during transformation of said solid prereduced material into steel, and wherein at least part of said combustible material is reacted with oxygen while still below the upper level of said mass of molten steel in said refining vessel, and wherein the amount of oxygen introduced into said refining vessel is sufficient to oxidize said thermogenic material and said portion of said combustible gas.

14. A method as defined in claim 2, wherein said jet of gaseous oxygen is introduced into said refining vessel through a lance orifice located in said refining vessel directed towards and upwardly spaced from said mass of molten steel.

15. A method as defined in claim 14, wherein said distance of said lance orifice from said molten mass of material in said refining vessel is adjustable.

## References Cited

## UNITED STATES PATENTS

|           |         |                |         |
|-----------|---------|----------------|---------|
| 2,889,219 | 6/1959  | Halley         | 75—52   |
| 2,962,277 | 11/1960 | Morrill        | 75—60 X |
| 2,978,318 | 4/1961  | Kalling et al. | 75—51 X |
| 3,153,588 | 10/1964 | Madaras        | 75—43 X |
| 3,356,490 | 12/1967 | Muller et al.  | 75—60   |

L. DEWAYNE RUTLEDGE, Primary Examiner

G. K. WHITE, Assistant Examiner

U.S. CL. X.R.